

## UNITED STATES PATENT OFFICE

2,337,943

## PROPELLENT POWDER PROCESS

Charles Earnest Silk, Alton, Ill., assignor to  
Western Cartridge Company, East Alton, Ill., a  
corporation of Delaware

No Drawing. Application December 3, 1938,  
Serial No. 243,767

14 Claims. (CL 52—20)

This invention relates to propellant powder and more particularly to an improved process for surface treating propellant powder grains in order to modify the characteristics thereof.

The object of this invention is to provide a process for the surface treatment of powder grains by means of which the treating agent is uniformly distributed among the grains under treatment, the absorption of treating agent by the grains may be made to occur as rapidly as desired, and the rate and extent of impregnation may be readily controlled.

In the course of the development of smokeless powders, a number of substances for improving the ballistic properties and/or storage characteristics have become known. These are generally substantially non-volatile compounds which are usually solvents for the smokeless powder base. Those agents which affect the burning rate of the smokeless powder are known as combustion modifiers and may be divided into two general classes: those which increase the potential and burning rate are known in the art as accelerators, and those which decrease the potential and burning rate are known as deterrents. Nitroglycerin, 25 nitroglycerol, and other nitric acid esters of polyhydric alcohols are examples of accelerators, while nitrohydrocarbons such as dinitrotoluene, high boiling esters such as alkyl phthalates, and substituted ureas such as dimethyl-diphenyl-urea are examples of deterrents. The stability and resistance to moisture absorption of powders may likewise be improved by the addition of an accelerator or deterrent, although substances are known which may be added to accomplish these results specifically, for example, diphenylamine for enhanced stability.

Such treating agents have been added to the smokeless powder base either during the manufacturing operation prior to the fabrication of the grains, as exemplified by the process described in British Patent No. 6,448 of 1892, or they have been added to the fabricated grains by a process of surface-treatment, for example, as taught in United States Patents No. 1,862,914 and No. 1,955,927.

In accordance with the process as described in the above mentioned United States Patent No. 1,955,927, surface treatment of powder grains may be accomplished by means of an emulsion or dispersion of a combustion modifier in water, or by means of an emulsion or dispersion of a combustion modifier solution in water. In the latter instance the combustion modifier was extended with a volatile solvent for the same which was

immiscible in water and a non-solvent for the smokeless powder base. It was found, however, that absorption of the combustion modifier from an emulsion or dispersion of such a solution of combustion modifiers was somewhat slower than the absorption in the case of a dispersion or emulsion of combustion modifier alone. In both cases there existed a tendency toward coalescence of the fine globules of combustion modifier, or combustion modifier solution, to produce larger globules than were desirable, with the result that the application of the treating agent was not uniform throughout the mass of grains being treated, and, in the case of large grains, was not uniform over the surface of the individual grains. While this tendency toward coalescence could be overcome by stabilizing the dispersion or emulsion as by use of a protective colloid, the presence of the protective colloid appeared to further increase the resistance toward absorption.

A more specific object of the present invention is to provide a process of surface treating propellant powder grains wherein absorption of the treating agent is facilitated and the tendency of protective colloids and/or volatile non-solvents for the powder grains to inhibit absorption, overcome.

Other objects will become apparent to those skilled in the art when the following description is read:

In accordance with the present invention absorption of surface treating agents by propellant powder grains is facilitated and accelerated, and in cases where the surface treatment is carried out in the presence of a protective colloid, or in the presence of a volatile solvent for the treating agent which is not a solvent for the powder grains, the tendency of those materials to inhibit absorption is overcome by the use of a relatively small quantity of volatile solvent which itself is a solvent for nitrocellulose. More specifically one phase of the present invention contemplates the application of treating agents to smokeless powder grains according to a procedure in which the treating agent is applied to the grains in the form of a dispersion or emulsion of a composite volatile solvent solution. In such case one component of the solvent is a water immiscible non-solvent for the smokeless powder base, while another component is a solvent for the smokeless powder base. During the treatment, the powder grains are advantageously maintained in suspension in the treating bath as by vigorous agitation. Uniform distribution of the treating agent among the powder grains and over the surfaces

of the individual grains is thus insured by the dilution or extension of the treating agent with a solvent and by maintaining such solution dispersed in the form of fine globules throughout the treating bath by adequate agitation. The use of a protective colloid may frequently be desirable to decrease the tendency toward coalescence of the dispersed globules of treating agent solutions, but even in such cases, where one component of the volatile composite solvent is a solvent for smokeless powder base, rapid absorption of the treating agent solution is accomplished.

The treating agent to be applied by the process of this invention may consist of combustion modifiers (either accelerators deterents, or both), stabilizers, or moisture-proofing agents, or a mixture of two or more such substances. Suitable accelerators are nitroglycerin, nitroglycol, and other nitric acid esters of polyhydric alcohols while nitrohydrocarbons such as dinitrotoluene, non-volatile esters such as alkyl phthalates, substituted ureas such as dimethyl-diphenyl-urea, and compounds of similar properties are suitable deterents. The quantity of treating agent to be added to the powder base usually amounts to less than ten per cent by weight of the finished product, although the quantity of an accelerator such as nitroglycerin may be as high as fifty percent.

In accordance with this invention where the treating agent is extended by solvent which is a non-solvent for the smokeless powder base, the treating agent is dissolved in a composite volatile solvent, one component of which is immiscible with water and is a non-solvent for the smokeless powder base, while another component is a solvent for the powder base. The volatility of the solvent mixture should be sufficiently high to permit the ready removal of the solvent from the grains following the surface-treatment and in general those with boiling points below about 150° C. have been found useful. As illustrating some of the suitable water-immiscible non-solvents may be mentioned aromatic hydrocarbons such as benzene or toluene, chlorinated hydrocarbons such as ethylene chloride or trichloroethylene, solvent naphthas, ethers such as isopropyl ether or normal butyl ether, and water-immiscible alcohols such as butyl or isobutyl alcohol. The quantity of such solvent that may be used with advantage depends on the quantity of treating agent it is desired to add to the grains, and may range from a weight equal to that of the treating agent when the latter amounts to fifty percent of the finished product to about ten to twenty times the weight of treating agent when one percent of the latter is being added.

To complete the formation of the treating agent solution, there is added a volatile solvent for the smokeless powder base such as ethyl or isopropyl acetate, acetone, ethyl methyl or methyl isobutyl ketone, or ethylene glycol diethyl ether in the case of pyrocollodion type of nitrocellulose, in an amount equal to 15% to 100% of the amount of the above described non-solvent which is used. The quantity of solvent for the powder base may be varied according to the particular solvent used, the desired rate of absorption, and the desired extent of penetration of the modifier in the powder grains. Both the rate of absorption and the extent of penetration are increased with increasing proportion of such solvent in the mixture. An excess of such solvent should generally be avoided since a tendency toward stick-

ing and agglomeration of grains is caused thereby, while a quantity substantially less than the stated minimum has no appreciable effect.

The solution of treating agent in the composite solvent may be emulsified by means of suitable agitation in water containing sufficient protective colloid to maintain the resulting fine droplets of solution in dispersed form until absorbed during the surface treatment of the powder grains. The treatment is preferably carried out by suspending powder grains in water by vigorous agitation and adding the solution of combustion modifier, or a preformed emulsion of combustion modifier solution, to the bath as agitation is continued. The treatment may be carried out at ordinary room or higher temperatures as desired, absorption of the droplets of treating agent solution being more rapid the higher the temperature. A temperature of 50° to 75° C. has been found to give good results.

As an illustrative embodiment of this invention, nitrocellulose powder grains in the form of spherical droplets 0.010 inch in diameter, resulting from the process described in U. S. Patent No. 2,027,114 to Olsen, Tibbitts, and Kerone, issued January 6, 1936, may be surface treated as follows:

300 pounds of powder grains are suspended by thorough agitation in 1200 pounds of water contained in a suitable jacketed vessel and hot water or steam is applied to the jacket so that the temperature of the powder-water suspension is raised to 65° C. To this suspension there is rapidly added an emulsion consisting of a solution of  $\frac{1}{2}$  pound of gum arabic in 120 pounds of water in which there has previously been dispersed, by means of vigorous agitation, fine globules of a solution containing 33 pounds of nitroglycerine, 33 pounds of toluene, 3.5 pounds of dinitrotoluene and 18 pounds of ethyl acetate. The dispersed globules of solution are thus uniformly distributed among the powder grains and their composition is such that they are completely taken up by the powder grains within fifteen minutes after the addition. In the absence of ethyl acetate or other nitrocellulose solvent which is highly fluid, similarly dispersed droplets of solution remain unabsorbed by the powder grains even after sixty minutes' agitation under the same conditions. When the desired extent of impregnation has been attained, as by continuing the agitation at 65° C. for thirty to sixty minutes, the suspension is cooled by passing cold water through the jacket. Less penetration of the treating agent into the grains may be secured by decreasing the quantity of nitrocellulose solvent, ethyl acetate in the present example, which is used. After being cooled, the powder grains are freed of excess water as by centrifuging, after which they are washed with cold water, and dried by means of air at 50° C. Finishing treatments, such as glazing with graphite, may then be applied according to known methods.

45 The stabilized aqueous emulsion of the solution of treating agent may be prepared with the use of one or more of the known suitable emulsifying agents as, for example, water-soluble gums such as gum arabic and gum tragacanth, dextrin, starch, water-soluble cellulose ethers such as methyl cellulose containing 22-26% methoxyl, casein, bentonite, alkali salts of sulfated higher alcohols, and the like. For best results, the quantity of emulsifying agent is adjusted so that separation into the component phases will occur in about 15 to 30 minutes after agitation has

stopped. If desired, a portion of the emulsifying agent may be added to the suspension of powder grains prior to the addition of the emulsion of the modifier solution.

Another example of a process embodying the principles of this invention comprises the surface-treatment of powder grains prepared by agglomeration of finely-divided particles of gelatinized nitrocellulose into clusters, which may range from 0.006 to 0.018 inch in average diameter, as described in the copending application of Olsen, Tibbitts and Kerone, Serial No. 620,332, filed June 30, 1932. The treatment is carried out in accordance with the procedure of the first example above, except that the added emulsion consists of finely dispersed globules of a solution containing 32 pounds of nitroglycerin, 32 pounds of toluene, 17 pounds of dibutyl phthalate, and 6 pounds of ethyl acetate in 120 pounds of water containing  $\frac{1}{2}$  pound of gum arabic. The reduction in the amount of ethyl acetate as compared with the first example is made in view of the presence in the solution of the phthalate, which is a good solvent for nitrocellulose.

In a third specific embodiment of this invention, 300 pounds of nitrocellulose powder grains as in the previous example may be suspended in 1,200 pounds of water at 15°-30° C. while this suspension is vigorously agitated, there is added a solution containing 77 pounds of nitroglycerin, 77 pounds of benzene, 7.7 pounds of dinitrotoluene, and 50 pounds of acetone. After 30 minutes' agitation, the temperature of the suspension is raised to 65° C., for example, by means of a suitable heating jacket. The coating treatment is complet after 90 minutes' agitation at 65° C. The acetone which is used in this treatment not only cuts down the time for complet absorption of the globules of modifier solution by the powder grains from ninety minutes at 65° C. to thirty minutes, but also has the advantage of causing the solution to disperse into finer globules than would result in its absence.

Even in cases where the treating agent may not be extended with a solvent of the character hereinbefore referred to, but where either the treating agent itself or the protective colloid employed in connection with the same has a strong tendency to inhibit absorption of the treating agent by the powder grains the addition of a small quantity, as for example, ten to fifty per cent on the weight of the treating agent, of a solvent which itself is a solvent for nitrocellulose may be incorporated with the treating agent with the result that absorption of the treating agent is accelerated. In such cases where no solvent which is not a solvent for nitrocellulose is employed, the solvent for nitrocellulose may advantageously be of the type which is not substantially miscible with water.

The process of this invention may advantageously be utilized for the application, by surface-treatment, of treating agents to any type, size or shape of smokeless powder base grains. Grains of partly or completely gelatinized nitrocellulose of any desired state of nitration which have been fabricated by any suitable process may be treated in accordance with this process and converted to a smokeless propellant powder having improved stability, resistance to moisture, enhanced progressivity of combustion, and/or higher potential. The surface-treatment of double-base powder grains, containing nitrocellulose and nitroglycerin, as well as of grains containing sub-

stitutes for nitrocellulose such as nitrostarch or other nitrated carbohydrates, is likewise included within the scope of this invention.

While in the foregoing description of the various embodiments of the invention, the vehicle in which the powder grains are suspended and in which the treating agent, or treating agent solution is dispersed or emulsified has been designated as water, it is to be understood that the invention is not limited to the use of water as the treating bath. On the contrary, it will be understood that any liquid vehicle which is not a solvent for the treating agent, and consequently a vehicle in which the treating agent, or treating agent solution, may be dispersed or emulsified in the form of globules, may be employed in lieu of water; provided, of course, that the chosen vehicle is not itself a solvent for the smokeless powder base. Consequently in interpreting the foregoing description and in construing the appended claims, the term "water" is intended as comprehensive of such other vehicles.

It will be understood, therefore, that the present invention is not limited to the specific details of the foregoing description, but on the contrary, that various modifications in the procedure and changes in the proportion of the ingredients and other details may be made by those skilled in the art without departing from the spirit of this invention. It is to be distinctly understood, therefore, that such modifications and the use of such individual features and combination of features as do not depart from the spirit of this invention are, although not specifically described herein, contemplated by and within the scope of the appended claims.

Having thus described the invention, what is claimed is:

1. In the art of manufacturing propellant powder, the process comprising, treating smokeless powder grains in a non-solvent bath with a dispersion of a solution, immiscible with the bath, composed of non-volatile combustion modifier in a composite volatile solvent containing a solvent for the powder grains and a non-solvent for the same and continuing the treatment until the treating agent is deposited upon the grains.
2. In the art of manufacturing propellant powder, the process comprising, treating smokeless powder grains in a non-solvent bath with a dispersion of a solution composed of non-volatile combustion modifier in a composite volatile solvent containing a solvent for the powder grains, and a non-solvent for the same, said non-solvent component of the solution being immiscible with the non-solvent of the bath and continuing the treatment until the treating agent is deposited upon the grains.
3. In the art of manufacturing propellant powder, the process comprising, treating smokeless powder grains with an aqueous dispersion of a water immiscible solution of combustion modifier in a composite volatile solvent containing a solvent for the powder grains and a non-solvent for the same.
4. In the art of manufacturing propellant powder, the process comprising, treating smokeless powder grains with an aqueous dispersion of a water immiscible solution of deterrent and accelerator in a composite volatile solvent containing a solvent for the powder grains and a non-solvent for the same.
5. In the art of manufacturing propellant powders, the process comprising treating nitrocellulose grains with a stabilized aqueous emulsion of

a solution of a non-volatile treating agent in a composite volatile solvent containing a solvent for nitrocellulose and a non-solvent for the same, which is immiscible with water and continuing the treatment until the treating agent is deposited upon the grains.

6. In the art of manufacturing propellant powders, the process comprising suspending smokeless powder grains in water, and adding to the suspension a stabilized emulsion of a solution of a non-volatile combustion modifier in a composite volatile solvent containing a solvent for nitrocellulose and a non-solvent for the same, which is immiscible with water and heating the mixture.

7. In the art of manufacturing propellant powders, the process of surface treating comprising, agitating smokeless powder grains in water containing dispersed globules of a non-volatile combustion modifier dissolved in a composite volatile solvent composed of a solvent for the powder grains and a water-immiscible non-solvent for the same, in the presence of a protective colloid and continuing the agitation until the treating agent is deposited upon the grains.

8. In the art of manufacturing propellant powders, the process of surface-treating smokeless powder grains comprising, dissolving a non-volatile combustion modifier in a mixed volatile solvent composed of a solvent and of a non-solvent for the powder grains to form a water immiscible solution, emulsifying the said solution in water containing an emulsifying agent, adding the said emulsion to an aqueous suspension of the powder grains and driving off the volatile solvent.

9. In the art of manufacturing propellant powders, the process comprising, treating nitrocellulose grains with an emulsion of a solution of nitroglycerin in a volatile mixed solvent comprised of a solvent and a non-solvent for nitrocellulose, said solution being immiscible with the other phase of the emulsion and said other phase being a non-solvent for nitrocellulose the said emulsion being stabilized by means of a protective colloid.

10. In the art of manufacturing propellant powders, the process comprising preparing a so- 45

lution of nitroglycerin, toluene and ethyl acetate, emulsifying the said solution in water containing a protective colloid, and treating nitrocellulose grains therewith in aqueous suspension.

11. In the art of manufacturing propellant powder the process comprising, preparing a solution of nitroglycerin, benzene, and acetone, emulsifying the said solution in water, and treating nitrocellulose grains therewith in aqueous suspension.

12. In the art of manufacturing propellant powder the process comprising, preparing a solution of nitroglycerin in a solvent mixture containing a component, which is a solvent for nitroglycerin but a non-solvent for nitrocellulose, and which is immiscible in water, and another component which is a solvent for both nitroglycerin and nitrocellulose, emulsifying the said solution in water containing a protective colloid, and treating nitrocellulose grains therewith in aqueous suspension.

13. In the process of surface treating smokeless powder grains wherein the powder grains are suspended in a water bath containing a stabilized emulsion of non-volatile liquid combustion modifier, the step of overcoming the tendency of the stabilized emulsion to inhibit absorption of the combustion modifier by the powder grains which comprises, adding a small quantity of a volatile liquid which is a solvent for both the powder grains and the combustion modifier.

14. In the process of surface treating smokeless powder grains wherein the powder grains are suspended in a water bath containing a stabilized emulsion of non-volatile liquid combustion modifier, the step of overcoming the tendency of the stabilized emulsion to inhibit absorption of the combustion modifier by the powder grains which comprises, adding a small quantity of a volatile liquid which is a solvent for both the powder grains and the combustion modifier, said volatile liquid being immiscible with the water phase of the emulsion.

CHARLES EARNEST SILK.